

## UNITED STATES PATENT OFFICE

1,939,616

## PULPBOARD

Hubert L. Becher, Trenton, N. J., assignor to  
The Agacote Millboard Company, Ewing Township,  
N. J., a corporation of New Jersey

No Drawing. Original application October 30,  
1928, Serial No. 316,109. Divided and this application  
December 11, 1930, Serial No. 501,669,  
and in Canada October 10, 1929. Renewed  
May 19, 1933

1 Claim. (Cl. 92—3)

My invention relates to a pulp board comprising a compressed mixture of fibres, paraffin, and Montan wax, a substantial portion of which is present in the form of a metallic salt of Montan wax, such paraffin and metallic salt of Montan wax being present in a uniform state of distribution and in a fine state of subdivision, which states are obtained when these substances are precipitated from an emulsion prepared from paraffin and saponified Montan wax.

Paraffin has heretofore been emulsified with the aid of an emulsifying agent, such as a resin soap or soap prepared from palmitic or stearic acid. I have found that a better and more suitable emulsion of paraffin, useful in the manufacture of molded pulp board, card board and paper, may be produced by the use of a soap made of Montan wax. An emulsion thus produced will retain its stability even in the presence of very large amounts of water. Pulp board, card board or paper sized with this emulsion is therefore very highly water-proof.

In the manufacture of my new pulp board in accordance with my invention I have obtained best results with pulp board which is made by beating paper pulp, wood pulp, or the like, in a beater, and then running such pulp into a mold and by means of pressure removing the majority of the water (see, for instance, United States Letters Patent No. 971,936, dated October 4, 1910, and No. 1,272,568, dated July 16, 1918), and subsequently drying out the remainder of the water by the application of heat.

My preferred method of preparing the emulsion for use with my new pulp board is to add from 20%—25% or more, by weight, of Montan wax to paraffin and then to add to the mixture an alkali, for instance, caustic soda, for saponifying the Montan wax in quantity sufficient to effect as complete a saponification of such wax as its nature will permit. The paraffin and the Montan wax are first melted in hot water and thoroughly agitated therein until they are broken up as finely as possible; the alkali is then added and the stirring is continued until substantially all the saponification has taken place and the paraffin has been thoroughly emulsified. The emulsion is then cooled with continued agitation until the paraffin has become hard. The amount of water used in this process should be sufficient to permit the formation of a proper emulsion but not much more than this amount. The mixture should be stirred at all times, stirring being particularly advisable during the cooling stage in order that the character of the emulsion may

not be destroyed by agglomeration and settling of the waxes.

Instead of diluting with hot water prior to cooling the emulsion, I may permit the emulsion to cool and during the cooling stage add cold water slowly so as to dilute the cooling emulsion gradually about in proportion to what otherwise would be the increase of its viscosity, and without suddenly chilling it. I may also instead of diluting the emulsion with either hot water or cold water pass it through a colloid mill suitably cooled, thus effecting the same result.

The emulsion may be used in the preparation of my pulp board either by mixing the same directly with the paper pulp, preferably in the beater, or by first converting it into an extremely fine suspension by effecting the double decomposition thereof with a metallic salt, for instance, magnesium sulfate or aluminum sulfate, thus rendering unnecessary the subsequent addition of a precipitant in the beater, the paraffin and the metallic salts of the saponified wax being so finely divided that the precipitant may be added at an early stage of the fibre treating process. The suspension, moreover, lends itself more readily to prolonged storing and does not "cream" as readily as the emulsion. In the case of an emulsion, if any paraffin should work its way up to the surface after the emulsion has been allowed to stand, slight agitation will easily restore homogeneity.

The precipitant, which may be added during the beating process, is the same material, for instance, magnesium sulfate or aluminum sulfate, by which the fine suspension referred to is produced. The suspension will thus contain the metallic salts of the saponified Montan wax which are produced when the emulsion is precipitated by the usual precipitants, namely, the metallic (f. i. aluminum) salt of the fatty acid (Montan wax) and the metallic salt of the alkali metal (f. i. sodium).

As Montan wax for some reason apparently not definitely known is not completely saponifiable, the saponified Montan wax, and the metallic salt of Montan wax, will contain a substantial admixture of an unsaponified ingredient or portion of the Montan wax.

A board thus produced is very highly water-proof and highly dielectric. The proportion of the combined waxes present in the emulsion or suspension to the weight of the fibre in the final product may vary within wide limits but is preferably from 1% to 5% or approximately  $\frac{1}{4}$  to 1.

part of Montan wax and from 1 to 4 parts of paraffin to 100 parts of fibre, dry weight.

*Example*

- 100 lbs. of Montan wax and 300 lbs. of paraffin are placed into 900-1000 lbs. of water heated sufficiently to melt both waxes and then thoroughly stirred. After the waxes have been broken up into fine particles, 7 lbs. of caustic soda in solution are added gradually and the heating and stirring are continued for 10-15 minutes after the addition of the caustic soda has been completed. The emulsion is then complete. In order to offset the increase in viscosity produced by the subsequent cooling, about 600-700 lbs. of water sufficiently hot to prevent chilling of the waxes are added and the emulsion is then allowed to cool below the melting points of the waxes and thus assume the form of a paste.
- To 1000 lbs. of fibre, in the beater, 40 lbs. of the emulsion are added, and after the fibre has been thoroughly beaten up, 2 lbs. of aluminum sulfate are added and the beating is continued until the

double decomposition of substantially all of the Montan wax soap has been effected. The fibre is then run into a mold, and subsequently processed to form the board in the manner hereinabove referred to.

The metallic salt of the alkali metal (f. i. sodium sulfate), being soluble in water, is washed out with the drainage water.

This application is a division of my application Serial No. 316,109, filed Oct. 30, 1928.

I claim:

Pulp board comprising a compressed mixture of about 1 to 4 parts of paraffin and from  $\frac{1}{4}$  to 1 part of Montan wax, a substantial portion of which is present in the form of a metallic salt of Montan wax, to 100 parts of fibre, such paraffin and metallic salt of Montan wax being present in a uniform state of distribution and in a very fine state of subdivision which states are obtained when these substances are precipitated from an emulsion prepared from paraffin and saponified Montan wax.

HUBERT L. BECHER.

80

85

90

95

100

5

105

0

110

5

115

0

120

5

125

10

130

0

135

0

140

0

145

70

150

75